

Patented July 31, 1923.

1,463,780

# UNITED STATES PATENT OFFICE.

HERBERT FROOD, OF CHAPEL-EN-LE-FRITH, ENGLAND, ASSIGNOR TO FERODO LIMITED, OF CHAPEL-EN-LE-FRITH, ENGLAND.

## COMPOSITION FOR COATING AND BONDING FABRICS.

No Drawing.

Application filed March 21, 1923. Serial No. 626,642.

To all whom it may concern:

Be it known that I, HERBERT FROOD, a subject of the King of Great Britain and Ireland, and a resident of Chapel-en-le-Frith, in the county of Derby, England, have invented certain new and useful Composition for Coating and Bonding Fabrics, of which the following is a specification.

This invention relates to a binder or filler for fabrics used for friction surfaces and wearing purposes.

The object of the invention is to provide an improved cementitious substance or binder for coating and bonding coated fabrics for frictional and wearing purposes.

According to this invention, a cementitious substance or binder for coating and bonding fabrics for frictional and wearing purposes, comprises dammar gum and rubber in suitable proportions. With the dammar gum and rubber, I may, if desired, incorporate other binding agents, such as e. g. those described in specifications of British Patents Nos. 4627 of 1909 and 164772, or the well-known phenol-aldehyde condensation products, glue, casein, chloronaphthalene substitution products, or sodium or potassium or other silicates or mixtures thereof, in about the proportion of one part of any, or a mixture of two or more, of such other binding agents to three parts of dammar gum and rubber.

Conveniently, the improved cementitious substance may consist of a mixture of approximately two parts of dammar gum and one part of rubber with suitable quantities of linseed or tung oil, a suitable drier and the other binding agent or agents when such is or are employed.

The following examples of the improved cementitious substance or binder have been found to give excellent results, the parts being by weight.

### Example 1.

|                                                      | Parts. |
|------------------------------------------------------|--------|
| Dammar gum                                           | 20     |
| Rubber                                               | 10     |
| Prepared linseed or tung oil                         | 20     |
| 50 Mineral naphtha, benzol or other suitable solvent | 50     |

### Example 2.

|                              | Parts. |
|------------------------------|--------|
| (a) Dammar gum               | 5      |
| Shellac                      | 4 55   |
| Alcohol (methylated spirit)  | 8      |
| (b) Dammar gum               | 20     |
| Rubber                       | 10     |
| Prepared linseed or tung oil | 20 60  |
| Trichlorethylene             | 50     |

With 100 parts of mixture (b) are incorporated 200 parts of mixture (a).

By the term "prepared oil", I mean oils prepared by the well known method of adding metallic driers thereto.

When the finished fabric is to be coloured, I may dye the fabric in the piece, or dye the yarn before weaving, or the fibres in the mass, and correspondingly colour the binder. Alternatively, the colouring of the finished fabric may be effected solely by the colouring of the binder.

The fabric may be coated with the binder under atmospheric or elevated pressure or in vacuo. Alternatively, the fabric may be coated by "frictioning" the binder into it, and I may employ any of the well known methods and means used in "frictioning" rubber and waterproofing compounds into fabrics. Conveniently, I may pass the fabric one or more times between rollers rotating at different speeds and apply the binder to that surface between which and the corresponding roller relative movement or slip takes place. The rollers may exert any desired pressure on the fabric to force the binder thereinto and consolidate same, and the frictioning may be effected under applied heat (in which case the rollers may conveniently be hollow and be heated internally by steam or otherwise suitably), or under the heat due to frictioning only.

After coating, the fabric may be air dried for a suitable period and be subsequently baked or stoved at a comparatively low temperature (e. g. about 160°-180° F.) for about 12 hours.

What I claim as my invention and desire to secure by Letters Patent is:-

1. A composition for coating and bonding

fabric consisting of dammar gum, rubber, a drying oil, and a solvent in substantially the following proportions, dammar gum two parts, rubber one part, oil two parts, solvent five parts.

2. A composition for coating and bonding fabric consisting of substantially two parts of dammar gum, substantially one part of rubber, substantially two parts of prepared linseed oil, and substantially five parts of a mineral hydrocarbon solvent.

3. As a new article of manufacture, a friction fabric consisting of a fabric base bonded and coated with dammar gum, rubber, a drying oil, and a solvent in substantially the following proportions, dammar gum two parts, rubber one part, oil two parts, and solvent five parts.

In witness whereof I have hereunto set my hand.

HERBERT FROOD.